

Oct. 20, 1931.

T. H. FROST

1,827,871

FINE EDGED BLADE

Filed Nov. 10, 1930



Fig.1.



Fig.2.



Fig.3.



Fig.4.



Fig.5.



Fig.6.

INVENTOR.

Thomas H. Frost.

By *Notary Public*

## UNITED STATES PATENT OFFICE

THOMAS H. FROST, OF CAMBRIDGE, MASSACHUSETTS

## FINE EDGED BLADE

Application filed November 10, 1930. Serial No. 494,591.

This invention relates to fine edged blades of ferrous alloys which may be hardened by the process of nitriding. In one aspect it comprises a novel blade of such alloy characterized by an elongated narrow nitrided area in which the cutting edge is included. In another aspect it comprises an improved method of producing such blades.

An important field of use of my invention is the production of safety razor blades of the thin flexible type which are adapted for use in holders wherein they are clamped for support. A nitrided blade of this character is disclosed in my copending application Serial No. 455,366 filed May 24, 1930, and in still another aspect the present invention constitutes a development or carrying forward of the invention therein disclosed.

The material I prefer to employ in the construction of the novel blade of my invention is an alloy of steel containing a substantial amount of aluminum, usually combined with chromium or molybdenum or tungsten and this I will refer to under the name "Nitralloy" by which it is commercially designated.

When such metal is exposed to ammonia fumes under conditions of high temperature it becomes nitrided upon its exposed surfaces and to a slight distance below its surface and is thereby rendered extremely hard and brittle. Attempts to use this material in the manufacture of fine edged blades have been unsuccessful prior to my earlier invention, partly on account of the fact that an expansion of the material takes place in the nitriding operation which warps or distorts the blank to an objectionable extent. Moreover, blades nitrided throughout their area have been too brittle for practical purposes. This has been particularly true of such an article as a flexible safety razor blade which is commonly maintained in a position of pronounced curvature when in use and must therefore be capable of withstanding appreciable bending. A razor blade of nitralloy completely nitrided is likely to shatter when bent between the fingers and become a menace to the user.

I have discovered that, if the nitrided area is confined to a narrow zone including

little more than the bevelled portion of the blank or the vertex of the cutting edge, then the blade as a whole, on account of its softer body portion, is rendered durable and capable of such flexing as is normally imposed upon safety razor blades. While the actual cutting edge is rendered extremely hard and somewhat brittle the more flexible tougher body of the blade offsets the fragility of its cutting edge. I have further discovered that a blade of this characteristic may be produced by beveling an edge of each blank and then, prior to the nitriding step, stacking the bevelled blanks so as to protect the bodies and expose the bevelled edges only thereof. By this procedure it is possible to produce blades in which the nitriding operation is confined to the bevelled portions which project from the sides of the stack in a slightly separated or spaced condition, whereas the engagement of contact between the flat faces of the blanks tends to prevent the entrance of ammonia and consequent nitriding of any substantial area within the cutting edge.

While I believe it is possible by insuring suitable conditions of pressure and flatness to stack the blanks for nitriding in the manner outlined, I prefer to employ spacing shims between adjacent blades and by employing shims of a non-nitriding material such, for example, as nitralloy shims already nitrided or shims of a non-ferrous metal, entrance of ammonia gas between the blanks is more effectively prevented.

The method of my invention, if preferred, may be characterized by the employment of shims plated with certain non-ferrous metals, for example, tin. When the stacked blades are separated by tin-coated shims the ammonia gas used in the nitriding operation is apparently prevented from reaching the adjacent faces of the stacked blanks by the action of the vaporized tin and a particularly clean cut zone of nitriding may be thus secured.

These and other features of my invention will be best understood and appreciated from the following description of its application to the manufacture of safety razor blades as

illustrated in the accompanying drawings, in which:

Fig. 1 is a view in perspective of a blade blank.

Fig. 2 is a similar view of the blank with roughly bevelled edges.

Fig. 3 is a view in perspective of a shim.

Fig. 4 is a view in perspective of a stack of blanks ready for the nitriding step.

Fig. 5 is a sectional view on the line 5—5 of Fig. 4, and

Fig. 6 is a view in perspective of a finished blade.

It will be understood that my invention is of general application to fine edge blades for all uses, although a most important field of use is in the manufacture of safety razor blades and its application to this field is herein illustrated.

In carrying out my invention a flat blank of the required shape is first produced. Such a blank 10 is shown in Fig. 1, having been punched or died out of thin sheet nitr alloy and coinciding in its dimensions to that desired in the finished blade. The blank is internally apertured, as by a slot 12, to receive the blade positioning elements of the holder and is provided with notches 14 at each corner to avoid corner cap pressure.

The material employed for the production of the blank may advantageously be of either of the following analyses:

| Element         | Analysis A | Analysis B |
|-----------------|------------|------------|
| Carbon.....     | .36        | .23        |
| Manganese.....  | .51        | .51        |
| Silicon.....    | .27        | .20        |
| Aluminum.....   | 1.23       | 1.24       |
| Chromium.....   | 1.49       | 1.58       |
| Sulphur.....    | .010       | .011       |
| Phosphorus..... | .013       | .011       |
| Molybdenum..... | .18        | .20        |

The analyses above set forth are typical of a satisfactory nitr alloy material for the manufacture of fine edge blades but nitr alloy of other similar analyses may be successfully used.

The next step in practicing the method of my invention consists in rough grinding the longitudinal edges of the blank to form a bevel 16. The formation of the bevels 16 is the first step in the production of the cutting edge and they are subsequently smoothed and sharpened as will presently appear.

The rough bevelled blanks are next stacked flatwise and secured in such position for the nitriding operation. As herein shown, I prefer to interpose a shim between adjacent blanks. Such a shim 18 is shown in Fig. 3. The shim is similar in shape to the blade blanks except that it is narrower by substantially the width of the bevel 16 so that when the blanks and the shims are stacked as shown in Figs. 4 and 5 the outer edge of each shim coincides with the inner line of the bevel 16. The result is that the bevelled edges of the

blanks project in spaced relation from the side surfaces of the stack, being wholly exposed while the body of each blank is enclosed and completely shielded by its engagement with the face of adjacent upper and lower shims. The shims 18 may be of copper, tin or other non-nitriding material or may be plated or otherwise coated with such material. As herein shown, I employ a steel shim having its opposite tinned faces.

The blanks with interleaved shims may be clamped in stack form in any convenient manner, but as herein shown, the stack is enclosed between a relatively thick bottom plate 20 and a relatively thick top plate 22 and the assembled pieces are clamped together by bolts 24 which pass through the plates, blanks and shims and are provided with nuts for subjecting the stack to the desired pressure.

Having arranged the blanks in stack form, as above outlined, or with the shims omitted, the stack is placed in a furnace and subjected to the action of ammonia gas for a predetermined interval of time and at a proper temperature for the nitriding requirements of the blade. Satisfactory blades may be produced from nitr alloy of the analyses above mentioned interval of time and at a proper temperature of from 900° F. to 950° F. or thereabout, for a period of two hours and under these circumstances a hard nitrided case will be formed upon the surface of the bevels 16 of the blank but nowhere else. This case may extend entirely through the material of the bevel or it may extend merely a few thousandths of an inch below the surface thereof but in any case the vertex of the blade is completely nitrided.

At the conclusion of the nitriding step the stack is removed from the furnace and allowed to cool. Thereupon the clamping bolts are released and the blades and shims separated. It will be found that a case of sufficient depth is formed to enable the rough bevel 16 of the blank to be finish ground, honed and stropped to produce the smooth bevel 17 of the finished blade 11 shown in Fig. 6. As already intimated, the elongated narrow nitrided zone defined by the bevel 17 in the finished blade is of extreme hardness and, although it is also brittle, it is carried by the un-nitrided soft and flexible body of the blade so that as a complete article the blade is durable and serviceable.

It will be noted that the rough grinding step produces a bevel 16 which approximates very closely the shape of the finished edge and presents a relatively thin zone for the nitriding operation. The rough grinding step may be effected rapidly since the material to be removed is relatively soft. The thin zone which is thereby produced is particularly well adapted to be efficiently nitrided since the depth of penetration required to form a completely nitrided cutting edge is reduced.

almost to a minimum. At the conclusion of the nitriding operation the rough beveled portion of the edge is brought to a fine, keen cutting edge by the finish grinding or otherwise smoothing. Here again an advantage of my improved process is apparent, for while there is a tendency to feather or form a wire edge in grinding the softer unnitrided material, the hard, brittle, nitrided material can be ground accurately or smoothed with no tendency to form a wire edge. In Fig. 6 the finish ground sharp cutting edge is indicated by reference character 17.

While I have herein referred to nitralloy as being a suitable and preferred material for the construction of blades in accordance with the novel method of my invention, the use of other ferrous alloys capable of being hardened by the process of nitriding is contemplated and would be within the scope of my invention.

Having thus described my invention, what I claim as new and wish to secure by Letters Patent of United States is:

1. A fine edged blade of a nitridable ferrous alloy bevelled to form a cutting edge, and nitrided only in the narrow area defined by the bevel of the blade.

2. A fine edged blade of a nitridable ferrous alloy having a cutting edge, and nitrided only in an elongated narrow area which includes said cutting edge.

3. A safety razor blade of a nitridable ferrous alloy, internally apertured to receive positioning means, having an exterior cutting edge and being nitrided only in a narrow area remote from its apertures and including the cutting edge.

4. A safety razor blade of a nitridable ferrous alloy, having a bevelled cutting edge and being provided with a nitrided case which includes the vertex of the bevel and a narrow zone adjacent thereto, the body of the blade being of relatively soft unnitrided material.

5. The method of making fine edged blades which consists in cutting out flat blanks of a nitridable ferrous alloy, beveling an edge of each blank, stacking the blanks so as to protect the bodies and expose the bevelled edges only thereof, and then nitriding the exposed edges.

6. The method of making fine edged blades, which consists in producing flat blanks of a nitridable ferrous alloy, rough beveling an edge of each blank, stacking the blanks under pressure, disposed face to face with their bevelled edges only exposed, nitriding the exposed edges, and sharpening the nitrided edges.

7. The method of making fine edges blades, which consists in producing flat blanks of the required shape, from a nitridable ferrous alloy, beveling an edge of each blank, stacking the blanks with interposed shims of such size as to maintain the bevelled edges in spaced

relation and to protect the body of each blank, and then nitriding the narrow zone of the projecting bevelled edges.

8. The method of making fine edged blades, which consists in providing flat blanks from a nitridable ferrous alloy, beveling an edge of each blank, interleaving the blanks with shims presenting non-ferrous contact faces and of such size as to maintain the bevelled edges in spaced relation, and then nitriding the bevelled edges of the blanks.

9. The method of making fine edged blades, which consists in stacking a series of nitridable bevel-edged blanks with interleaved shims of non-nitriding material, the shims terminating within the bevelled edges of the blanks thus exposing them in spaced relation, and then nitriding said exposed edges.

10. The method of making blades, which consists in stacking a series of nitridable bevel-edged blanks with interleaved shims having tin-coated surfaces, and exposing the stack to the action of ammonia gas under conditions of high temperature, thus nitriding the narrow bevelled areas only of the blades.

11. The method of making safety razor blades, which consists in stacking flat, nitridable, bevel-edged blade blanks in alternation with tin-coated shims of less width than the blanks, exposing the stack to the action of ammonia gas under conditions of temperature sufficiently high to vaporize a portion of the tin from the shims thus hardening the bevelled portions of the blanks, and finally finish grinding the bevels to complete the blades.

12. A nitralloy safety razor blade having a relatively soft tough body of unnitrided nitralloy, and a narrow marginal zone which is nitrided and therefore hard and rust-resistant and in which the cutting edge is formed.

13. The method of making fine edged blades from a nitridable ferrous alloy, which consists in rough grinding the edge of the blade blank to form a bevel of the approximate shape desired, then nitriding the blank in an area including said beveled portion, and finally finishing the nitrided beveled portion to form a keen cutting edge.

14. The method of making safety razor blades of a nitridable ferrous alloy, which consists in rough grinding the edge of the blade blank to form a bevelled portion of approximately the desired shape, nitriding the beveled portion while protecting the body of the blank against nitriding, and finally smoothing the nitrided bevelled portion by removing sufficient nitrided material to form a fine cutting edge.

Signed at Boston, Massachusetts, this 8th day of November, 1930.

THOMAS H. FROST.